

## UNITED STATES PATENT OFFICE

2,155,348

## ALLOY STEELS

Marcus A. Grossmann, Chicago, Ill., assignor to  
United States Steel Corporation, New York,  
N. Y., a corporation of New Jersey

No Drawing. Original application October 22,  
1936, Serial No. 107,104. Divided and this ap-  
plication January 26, 1939, Serial No. 253,019

3 Claims. (Cl. 75—123)

The present invention relates to alloy steels.

This application is a division of the application  
for United States Letters patent filed by the  
present applicant on October 22, 1936, Serial No.  
107,104.

5 In the strict sense, steel may be said to be an  
alloy of iron and carbon. However, in a metal-  
lurgical sense, in which the term is used in this  
specification, an alloy steel is steel (that is—iron  
10 and carbon) alloyed with another chemical ele-  
ment or other chemical elements.

An object of the present invention is to pro-  
duce an alloy steel which is well adapted to re-  
sist failure by fatigue, especially for use in highly  
15 stressed parts, such as springs.

15 A further object is to produce an alloy steel for  
general purposes which involves no special equip-  
ment in its manufacture and which has im-  
proved characteristics over steel as heretofore  
20 known and used.

20 A further object is to provide a steel well  
adapted for use in cushioning springs, which steel  
will effectually resist deterioration in service.

25 A further object is to provide an alloy steel in  
which the characteristics of titanium are utilized  
to advantage in the manufacture of alloy steels.

30 A further object is to provide an improved  
steel well adapted to meet the needs of com-  
mercial operation.

35 Further objects will appear as the description  
proceeds.

The present invention contemplates the accom-  
plishment of the objects above referred to by  
35 providing a shallow hardening alloy steel. To  
the skilled steel manufacturer the term "shallow  
hardening alloy steel" has a definite significance,  
meaning a steel which, when heated to above its  
critical temperature and then cooled, has a rela-  
tively pronounced tendency to change rapidly  
40 from the austenitic to the pearlitic type of in-  
ternal structure. Steel of fine grain structure  
tends to be shallow hardening, though of course  
certain alloy steels, even though they be fine  
grained, may not be shallow hardening in com-  
45 parison with the steels for which invention is  
claimed herein. Of course, it is possible to pro-  
duce shallow hardening steel by using a very  
restricted amount of carbon, and such steel has  
its uses in the arts. The present invention,  
50 however, is limited to steels in which the carbon  
content is equal to or greater than .45% by  
weight.

55 In defining the degree of shallow hardening  
contemplated in the present invention it may be  
observed that certain alloy steels, as for exam-

ple nickel chromium steel, have characteristics  
differing from steels contemplated in the pres-  
ent invention. As is well known, alloy steels as  
ordinarily known to metallurgists will, when  
heated to a temperature of say 1600 deg. F., form  
austenite, which is understood by metallurgists  
to be a solution of carbon in iron. As the steel  
is cooled from the temperature referred to, the  
structure changes, and when the steel reaches the  
neighborhood of about 900 deg. F. there is a 10  
tendency to form pearlite, which is a tough sub-  
stance of low hardness. In the case of most al-  
loy steels as now known and used, as for example  
the nickel chromium steel above referred to, the  
length of time in the temperature zone in the 15  
neighborhood of 900 deg. F. required for the  
formation of pearlite is in the neighborhood of  
20 seconds. The temperature zone referred to  
may range from 1050 to 850 deg. F. In the case  
of the alloy steels forming the subject matter of 20  
the present invention, the period of time required  
in the 900 deg. zone referred to is in the neigh-  
borhood of 8 seconds. Considering a body of  
steel which has been heated to say about 1600  
deg. F. and quenched in water, it will be readily 25  
understood that in the case of nickel chromium  
steel or the like the period of dwell in the 900 deg.  
zone referred to may be too short to form pearl-  
ite, but said period of dwell may be ample for  
the formation of pearlite in the composition of 30  
shallow hardening steels. In other words, using  
the example above referred to, the period of time  
in which the center of the member under test is  
in the temperature zone of 900 deg. F. above re-  
ferred to may be less than 20 seconds but more 35  
than 8 seconds. In the event that pearlite has  
not formed in the quenching operation, the al-  
loy steel, upon further cooling, will form mar-  
tensite, which is a hard material. In the event  
that pearlite has formed in the center of the 40  
member under test in the quenching operation,  
this pearlite will retain its identity when the  
member under test has cooled to atmospheric  
temperature. The above example illustrates a  
measure which may be applied to define the de-  
gree of hardenability contemplated in the pres-  
ent invention. For convenience, the measure of  
hardenability may be expressed in connection  
with an alloy steel bar. The present invention  
contemplates a composition of alloy steel such 45  
that when a cylindrical bar of 1½ inches or  
more in diameter of homogeneous composition  
is heated to a temperature of approximately  
1600 deg. F. and then quenched in still water at  
room temperature, the material at the axis of 50  
55

said bar will, upon cooling to room temperature, have a Rockwell hardness of not more than 50-C. Expressed in another way, and referring to the quenching of the alloy steel in oil, the present invention contemplates a composition alloy steel such that when a cylindrical bar of 1 inch or more in diameter of homogeneous composition is heated to a temperature of approximately 1600 deg. F. and then quenched in still oil at room temperature, the material at the axis of said bar will have a Rockwell hardness of not more than 50-C.

It will be understood, of course, that the references immediately above made to bars of specified diameters are merely for convenience of definition of one property of these steels. The steels, of course, are useful in members of all dimensions including small sections in which the steels harden through to their axes or midsections.

Titanium has the advantage that it produces fine grain structure and is relatively low in price. As is well known, the cheapest form of titanium on the market at the present time is that which has been reduced by treatment with carbon resulting in what is known as a high carbon ferro titanium. In some arts, the high carbon content is objectionable but in the manufacture of alloy spring steel in which the carbon content is relatively high, the high carbon content of the low priced high carbon ferro titanium is not objectionable.

Titanium has the advantage that it tends to produce fine grain structure and shallow hardening over a relatively wide temperature range in the hardening operation. Moreover, when using titanium in the manufacture of alloy spring steel the amount of aluminum may be materially reduced from present practice in the melting operation to secure fine grain structure and shallow hardening.

In carrying out the present invention it is contemplated to use in the manufacture of the improved alloy steel a predominating amount of titanium either with or without other shallow hardening elements, such for example as vanadium or equivalent. Correspondingly, the present invention contemplates a relatively low amount of the deep hardening elements (such for example as manganese, chromium and/or nickel). The relative terms referred to in the preceding sentence have reference to the functions of the alloying elements referred to as commonly used in alloy steels in common use today.

Proceeding to a more specific definition of alloying elements contemplated in the present invention, the following observations may be made:

Since titanium reaches its full effectiveness for grain refinement at approximately 0.06% by weight, a predominating amount of titanium in the alloy steel according to the present invention would be approximately 0.02 to 0.06% by weight.

Since vanadium reaches its full effectiveness at about 0.15% to 0.20%, a predominating amount of vanadium would be about 0.075 to 0.20% by weight.

On the other hand, chromium may be said to have its greatest effectiveness at about 1.5% by weight, so that a predominating amount of chromium would be about .75%-1.5%.

Since manganese reaches its maximum effectiveness at about 2% by weight, a predominating amount of manganese would be about 1.25%-2% by weight.

Since nickel reaches its full effectiveness at about 3% to 4%, a predominating amount of nickel would be about 1%-4% by weight.

Therefore, expressing the purpose of the present invention in other language, it may be said that the present invention contemplates the use of titanium in the amount of 0.02 to 0.06% by weight, said element being used without chromium or manganese if preferred; or, if chromium be used, then with less than .75% by weight of chromium; or, if manganese be used, then with less than 1.25% of manganese. Expressed in still other language, certain advantages of the present invention will be had if the shallow hardening elements (for example titanium, with or without vanadium or equivalent) are used to a percentage equal to at least 50% of their fully effective amount in opposing hardening in quenched steels; and certain advantages of the present invention will be had if the deep hardening elements (for example chromium, manganese and/or nickel) are restricted to not more than 50% of their fully effective amounts as hardening agents in quenched steels. Another way of defining the limits of the materials contemplated in the present invention is by reference to the "critical cooling rate" of the materials. Critical cooling rate of steels may be defined as that rate above which a steel will harden in the cooling process and below which a steel will not harden. When the term "harden" is used in this connection it is intended to convey the meaning that the material of the steel becomes the hard material "martensite". The present invention contemplates steels which when quenched in a quenching medium at atmospheric temperature will just harden if it passes 1325 deg. F. at a rate above 50 deg. per second but below 150 deg. per second.

Those skilled in the art will understand that manganese is usually present in the manufacture of steel to the extent of about .2%-.5% by weight, since manganese is commonly used as a de-oxidizer in steel making; and for the same reason silicon is usually present in amounts of about .2%.

Proceeding now to a still more specific recitation of analysis of steel falling within the scope of the present invention, the following example may be recited:

|                                                 | Per cent   |
|-------------------------------------------------|------------|
| Carbon, from                                    | .85 to .95 |
| Manganese, from                                 | .20 to .50 |
| Silicon, from                                   | .10 to .35 |
| Chromium, from                                  | .20 to .50 |
| Titanium, from                                  | .03 to .06 |
| Balance largely iron with traces of impurities. |            |

It will be understood, of course, that the analysis just noted is illustrative only, and the objects of the present invention may be realized by proper balancing of shallow hardening elements against deep hardening elements. For example, the carbon may vary from .45% to 1%; the manganese may vary from .40% to 1.25%; the chromium may vary from 0 to .75%; the titanium may vary from 0.01% to 0.10%. A choice of the elements referred to, to provide a shallow hardening steel meeting the tests recited in this specification, will fall within the scope of this invention.

Anyone familiar with the manufacture of alloy steels has readily available to him information as to the constituents and the amounts thereof which must be used in producing the steels having the foregoing analyses.

In arriving at the object of making a shallow hardening alloy steel, the present invention contemplates a steel of fine grain size. In referring to fine grain size it is to be understood that reference is had to the grain size of austenite, which is the structure composing the steel when the steel has been heated to a high temperature (for example 1600 deg. F.) preparatory to hardening by quenching. The term "fine grain" or "fine grain size" as used in this specification means from #5 to #8 on the ASTM chart of grain sizes. This may be further explained as meaning more than 12 grains per square inch when examined at a magnification of 100 diameters.

The fact is well known that fine grain size tends to shallow hardening. It is also well known that very fine grains, particularly #7 and #8, according to the ASTM chart, exhibit structural features known as abnormality, meaning thereby a particular distribution of the iron carbide (that is—cementite) observed in the carburizing test (McQuald-Ehn carburizing test), which test is sometimes used in determining grain size.

In order to arrive at fine grain size (including abnormality) it has been common to add, in the furnace, in the ladle or in the molds, about one pound of aluminum per ton of steel. It has been discovered that if titanium be used as one of the shallow hardening elements, the amount of aluminum may be materially reduced. Titanium tends to produce fine grain structure and shallow hardening in steel over a relatively wide temperature range in the hardening operation.

As is well known, silicon is used in the manufacture of alloy quality steels for the purpose of combining with the oxygen and thereby removing said oxygen. An excess of silicon always appears in the finished steel of this type and may properly be considered to be a trace of impurity. Accordingly, in the appended claims the term "traces of impurities" will include this excess silicon.

The alloy steels forming the subject matter of this invention are characterized by a high degree of ductility, toughness, resiliency and resistance to shock and fatigue.

Though certain preferred analyses and steps have been recited in the foregoing specification, many modifications will occur to those skilled in the art. It is intended to cover all such modifications that fall within the scope of the appended claims.

What is claimed is—

1. An alloy steel characterized by a high degree of resilience and resistance to shock and fatigue which is composed of the following ingredients within the ranges specified and balanced against each other to produce a shallow hardening steel:

|                 | Per cent    |    |
|-----------------|-------------|----|
| Carbon, from    | .45 to 1    | 15 |
| Manganese, from | .40 to 1.25 |    |
| Titanium, from  | .01 to .10  |    |

remainder iron with traces of impurities.

2. An alloy steel which is fine-grained and is composed of the following ingredients substantially in the amounts specified:

|                 | Per cent   |    |
|-----------------|------------|----|
| Carbon, from    | .60 to .70 | 25 |
| Manganese, from | .70 to .90 |    |
| Titanium, from  | .03 to .06 |    |

balance iron with traces of impurities, said steel being characterized by a high degree of ductility, toughness, resiliency and resistance to shock and fatigue.

3. An alloy steel which is fine-grained and is composed of the following ingredients substantially in the amounts specified:

|           | Per cent |    |
|-----------|----------|----|
| Carbon    | .65      |    |
| Manganese | .80      |    |
| Titanium  | .04      | 40 |

balance iron with traces of impurities, said steel being characterized by a high degree of ductility, toughness, resiliency and resistance to shock and fatigue.

MARCUS A. GROSSMANN.

45